

# UNITED STATES PATENT OFFICE.

FRANZ MERKEL, OF OFFENBACH-ON-THE-MAIN, GERMANY, ASSIGNOR TO CORPORATION OF CHEMISCHE FABRIK GRIESHEIM-ELEKTRON, OF FRANKFORT-ON-THE-MAIN, GERMANY.

## PROCESS FOR DYEING PELTS, HAIRS, FEATHERS, AND THE LIKE.

1.175.539.

Specification of Letters Patent. Patented Mar. 14, 1916.

No Drawing.

Application filed April 22, 1915. Serial No. 23,075.

*To all whom it may concern:*

Be it known that I, FRANZ MERKEL, a citizen of the German Empire, and resident of Offenbach-on-the-Main, in the Grand Duchy of Hesse, Germany, with the post-office address Landgrafenring 7, have invented new and useful Improvements in Processes for Dyeing Pelts, Hairs, Feathers, and the like, of which the following is a specification.

10 I have found, that by means of meta-oxy-  
diphenylamin valuable brown dyeings are  
obtained on pelts, hairs, feathers and the  
like by treating the pelts, etc., mordanted or  
not, with a solution of meta-oxydiphenyl-  
amin, adding an oxidizing agent. The thus  
obtained dyeings possess a great fastness to  
light and differ from those dyeings hitherto  
obtained on the mentioned materials, by not  
having the reddish tinge of those dyeings.  
15  
20 Moreover they have the characteristics of  
natural skins, and therefore are valuable  
for the production of imitations of natural  
pelts.

25 The following example illustrates the invention: Raw skin or skins prepared in the usual way, for example, by washing, followed by treating the ends of the hair with alkalis, are introduced for about 6 hours into a mordant, consisting of a solution of 30 3 grams of bichromate of sodium and 2 grams of sulfate of copper per liter. Subsequently the skins are introduced into the real dye-bath consisting of: for instance 1.5 to 3 grams of meta-oxydiphenylamin, 1.25 to 2.50 c. c. m. caustic soda lve (28 per cent.), 35 1 liter of water. Immediately about 25 c. c. m. of bichromate-solution (1:10) are added, and then about 1 to 2 grams of perborate of sodium. In the so produced liquid 40 the skins are at first well handled and after

about half an hour, about 5 c. c. m. of formic acid (1:10) are added, the skins being well handled meanwhile until the liquid does not prove alkaline any more by testing on test-paper, but shows a nearly neutral or only 45 a little acid reaction. The skins are kept in the liquid referred to for a considerable time, for example during an entire night, and are handled from time to time; they are then taken out, washed well, centrifuged 50 and finished in the usual manner. A beautiful deep brown of a very good fastness to light is obtained.

In the place of a solution of bichromate and perborate of sodium there can be used other oxidizing agents for instance a solution of hydrogen peroxid. 55

In the same manner hairs, feathers and the like can be dyed.

Now what I claim and desire to secure by <sup>60</sup> Letters Patent is the following:

1. Process for dyeing pelts, hairs, feathers and the like which comprises treating the material to be dyed in a solution of metoxydiphenylamin containing an oxidizing agent. 65

2. Process for dyeing mordanted pelts, hairs, feathers and the like which comprises treating the mordanted material to be dyed in a solution of meta-oxydiphenylamin containing an oxidizing agent, substantially as described. 70

That I claim the foregoing as my invention, I have signed my name in presence of two witnesses, this first day of April, 1915. 75

## FRANZ MERKEL.

**Witnesses:**

JEAN GRUND,

## CARL GRUND.